

Jan. 18, 1938.

W. E. WAGNER

2,105,993

SHOT SHELL

Original Filed June 24, 1929

Fig. 1.



Fig. 2.



Fig. 3.



Fig. 4.



Fig. 5.



Inventor:  
WILLIAM E. WAGNER,  
By John N. Rumminger  
His Attorney.

## UNITED STATES PATENT OFFICE

2,105,993

## SHOT SHELL

William E. Wagner, Kilworthy, Ontario, Canada,  
assignor to Western Cartridge Company, East  
Alton, Ill., a corporation of Delaware

Application June 24, 1929, Serial No. 373,127  
Renewed May 3, 1937

8 Claims. (Cl. 102—15)

This invention relates to cartridges, and more particularly to shot shells adapted for use in shot guns.

In a shot shell the propellant charge is confined by wadding, over which is placed the shot charge and the latter is in turn confined by its covering wad and the turned over end or crimp of the paper shell, while a primer is provided in order to ignite the powder. The wadding does not, however, form such a tight seal as does the bullet in a rifle; accordingly, the conditions encountered in a rifle cartridge and in a shot shell are entirely different. Where quick burning powder is used, a high and rapidly rising initial pressure is applied to the shot charge, causing rapid acceleration thereof followed by rapid falling off in acceleration during the subsequent stage. In order, therefore, to produce a high muzzle velocity, it has been heretofore deemed necessary to employ charges of powder sufficient to produce high initial pressures; the latter are, however, necessarily limited by the limiting breech pressure. These conditions have to a large extent been overcome by the employment of coated or impregnated powder securing a progressive burning of the powder charge by retarding the initial combustion rate. In such a progressive burning powder, the combustion at the surface will start the shot charge on its course at a lower pressure while the maximum pressure is developed an extended distance along the gun barrel; this latter is due to the increased rate of combustion of the powder grains after the coating or impregnation has been consumed.

Coated powders as commonly used in shot shells are dense nitro-cellulose powders of high nitration coated with a deterrent. Not only are such coated powders more difficult to ignite than double base powders, such as nitro-cellulose-nitro-glycerin powders, but they are more hygroscopic and under varying climatic conditions may be more subject to changes in burning rate. The ballistic properties and characteristics of coated powders may, therefore, be affected by storage under varying climatic conditions. These conditions cannot be fully met to the desired extent by variation of the primer charge, but the irregularities may, in fact, be increased. On the other hand, uncoated double base fast-burning powders do not have the desired progressive burning action when employed in shot shells as now constructed.

A powder charge starts to burn from the outer surfaces of the individual grains while sufficient pressure is being built up to overcome the inertia of the shot charge and start it; the combustion then continues to the centers of the grains as the shot charge moves along the barrel. Accordingly, in a shot shell having a standard base and loaded with a propellant charge of readily ignitable powder and with regular primers such as have been found most suitable to ignite such powders under different storage conditions, the combustion does not start merely from a layer near the base, but the combustion proceeds and the gases are evolved from a small quantity of powder burning from the surface of grains throughout substantially the entire powder charge. This is even true of a shell provided with a base wad having a cavity or well of reduced diameter in front of the primer and even flared or stepped, unless the cavity or well is constructed as hereafter described. The purpose of such a base wad as heretofore constructed has really been to partly fill the powder space in the shell and make the same available for dense powders without the addition of extra wads between the powder and shot charges, in order that the standard length of the shell might be maintained. Even in such shells, however, the primer flame permeates substantially the entire powder charge; accordingly, where fast burning powder is used even in such a shell, the ignition and the pressures produced will not differ substantially from those produced in shells having no cavity in the base, and high velocities cannot, therefore, be attained without dangerously high breech pressures.

In a shot shell, therefore, it is the rate of evolution of the gas which controls the initial pressure as well as the final velocity of the shot charge. In a shell employing a progressive burning powder of the coated or impregnated type the initial combustion rate is retarded by the coating or impregnation on each grain, so that the initial pressure can be maintained fairly low while the working pressure is sustained an extended distance along the gun barrel.

One of the objects of this invention, therefore, is to provide a loaded shot shell in which the initial combustion rate of the propellant charge is retarded sufficiently to develop a low maximum pressure an extended distance along the gun barrel, while the pressure is sustained to produce a high average pressure, and which has improved features and characteristics.

Another object is to develop a process of controlling the ballistics of such a loaded shot shell in a simple and effective manner.

Another object is to provide a shell and process

5 10 15 20 25 30 35 40 45 50 55

whereby the ignition of the charge is facilitated but in which the initial pressure is kept down while the pressure is sustained even after the shot charge moves out of the shell.

5 Another object is to provide a shot shell employing a fast burning powder, such as a double base powder, in which the shell, and particularly the base thereof, is so constructed and co-ordinated with the powder as to produce a progressive 10 burning action when fired in a shot gun.

Further objects will appear from the detail description, taken in connection with the accompanying drawing, in which—

15 Figure 1 is a longitudinal section through a shot shell having a stepped recessed base;

Figures 2, 3 and 4 are views similar to Figure 1, but showing the dimensioning of a base wad well in accordance with this invention;

20 Figure 5 is a diagram, showing the relation of pressures along the gun barrel in the shells, Figures 1, 2, 3 and 4.

A number of embodiments of this invention will now be described; it is, however, to be understood that these are merely given as examples, 25 as this invention is susceptible of various other embodiments.

Referring to the accompanying drawing, the shot shell generally, except as hereinafter described, may be of the usual form, comprising a 30 tube 1, which may be of paper, a metallic base 2, a base wad 3, and a primer in the form of a battery cup 4. The charge of propellant 5 is shown as confined by wads 6 and 7, the wad 6 being generally of cardboard, while the wads 7 are of the compressible type, such as felt wads. The shot charge 8 is confined by a wad 9 secured by a crimp 10. The cartridge or shell so far generally described may be of any suitable or usual construction and, as shown, is of 12 gauge.

40 Referring now to Figures 1 to 4, the base wad 3 is shown as recessed to provide a cavity or well 11 in front of the primer, and this well may terminate in a flared part 12, which may be stepped, as shown, and provided with a suitable angle of 45 flare. In accordance with this invention, however, the well 11, which contains a part of the propellant charge, is so dimensioned as to substantially retard the initial combustion rate of the propellant charge. This well is, therefore, 50 dimensioned with reference to the characteristics of the propellant in order to control the ballistics of the shell. The well diameter is, therefore, contracted sufficiently and its depth extended sufficiently, with reference to the normal rate of 55 ignition of the propellant, in order to control the pressure generated by the charge. Figures 1 to 4 show wells of progressively decreasing diameters and of progressively increasing depths; this, as hereinafter described, has a marked effect upon the ballistics of these shells. A practical example and a method of determining the dimensions 60 of the well will be hereinafter more fully described; but at this point it will be well to describe the action of the combination, reference 65 being particularly had to Figure 4.

As the primer gases issue from the flash hole of the primer, they are restricted in the confined space in the well filled, as it is, with powder 70 grains. The enclosing walls of this well take up the impact of the primer gases, which are deflected by the powder grains between the wall of the well and the flash hole of the primer. For very fast burning powders, the well is made narrow and deep, the diameter being, of course, de-

pendent upon the granulation of the propellant; for the diameter must be sufficient to permit free admission of the powder grains in loading and permit escape of the primer gases from the flash hole of the primer. The primer gases issuing 5 from the flash hole are, therefore, not only deflected and muffled by the walls of the well, but also by the powder grains therein. The result is, therefore, that the penetration of the charge by the primer flame is restricted so that the initial 10 ignition is practically confined to the charge within the well and adjacent the base of the shell. The checking of the primer gases further serves to confine their energy content largely within the well, resulting in improved ignition of the 15 powder contained therein.

As a result, therefore, the initial combustion is restricted to a part of the propellant charge, more particularly that part in and adjacent to the well, so that the ignition of the charge is retarded. Thereafter the ignition of the body of the propellant proceeds under the combined action of the primer gases and the gases evolved by the combustion of that portion of the powder charge in and adjacent to the well. The pressure and 20 temperature, therefore, rise gradually as the charge progressively ignites and burns, so that the velocity of the shot charge moving out of the shell is built up gradually. However, pressure and temperature are maintained not only as the 25 shot charge moves out of the shell, but also as it moves for an extended distance along the gun barrel. The propellant charge, therefore, does not burn rapidly to produce a high initial pressure, as in other shells when equal charges of 30 fast burning powders are used, but the pressure is gradually built up and sustained for an extended distance along the gun barrel. On the other hand, by employing a fast burning powder, in which, however, the penetration by the primer 35 flame is restricted to retard the initial combustion, both pressure and temperature are sustained as the shot charge moves out of the shell; for the propellant in front of the well is ignited by the combined action of the primer gases and the 40 gases evolved by the combustion of that portion of the charge in and adjacent to the well; furthermore liability of failure of ignition of the forward part of the charge is obviated by the use of a fast burning powder. Moreover, the primer 45 charge can be increased to secure the desired ignition on account of the fact that the penetration of the charge by the primer flame is restricted.

Since the penetration of the primer gases is 55 restricted by deflection from the grain surfaces in the well against the walls of this well, additional control of the ballistics may be secured by proper selection of the granulation of the powder charge, particularly that portion in the well. The primer gases issuing from the flash hole of the primer under high velocity are conceivably more retarded and deflected from a direct course by large grains than by small grains; accordingly as the deflected gas currents meet other large 60 grains of powder, they will be further retarded and deflected sideways and back and penetrate less deeply into the main powder charge than is the case with finer grains, which furnish a more direct course through the body of the powder. There is, of course, a limit to this action; for if the powder is extremely fine, it will, when compressed, act somewhat like a solid mass, thereby preventing penetration of the ignition 70 gases altogether; this phase can, however, be dis-

- regarded, for such a closely packed fine powder results in such poor ignition and low velocities as to be impractical. In accordance with another embodiment of this invention, therefore, the well 5 may contain powder of a larger granulation than the main body of the charge; this granulation being selected with reference to the normal rate of ignition of the propellant and the dimensions of the well as determined. It will, therefore, be seen 10 that by proper dimensioning of the well and by proper selection of propellant grains therein, the penetration of the charge by the primer flame may be restricted to the desired extent to substantially retard the initial combustion as de- 15 sired.

In the shot shell embodying this invention, the velocity is mainly determined by the quantity of the propellant charge, while the pressure is adjusted by the dimensioning of the well and the 20 granulation of the powder therein. Within limits the pressure is reduced by decreasing the diameter or increasing the depth of the well or by increasing the grain size of the powder in the well; and the pressure can be controlled by variation 25 of any or all of these factors. It will be understood, of course, that any well will not necessarily have a controlling effect, but adaptation is required, particularly with reference to the character of the propellant.

30 It will be well at this point to describe a practical method of determining the dimensions of the well with reference to the characteristics of the propellant to be used and the shot charge. Taking a fast burning double base propellant, 35 such as Hercules No. 2 (a nitro-cellulose-nitro-glycerin powder containing 30% of nitro-glycerin and whose grain is a flat disc .055 inch in diameter and .005 inch thick), for use in a 12 gauge shot shell containing, for instance, 1 1/4 oz. of 40 No. 6 shot, the procedure can be as follows: Let us take, say arbitrarily, a shell formed with a well in the base wad and dimensioned as shown in Figure 3. A number of such shells are now 45 loaded, each with an arbitrary trial charge of the chosen propellant and with the desired shot charge and suitably wadded. These shells are now fired and tested to determine the velocity and also the pressure. If the velocity is higher or lower than desired or necessary, the propellant 50 charge is decreased or increased respectively and another batch of such shells is loaded with the revised charge. After the propellant charge required to produce the desired velocity has thus been determined, the pressure may be greater 55 than desired; in fact, unless the base has been specially adapted and dimensioned for the propellant, the pressure will be above the desired limit with a fast burning powder. The procedure is, therefore, to increase the depth or decrease the 60 diameter of the well or alter both until further tests show that the pressure has been reduced to the desired value. Of course, if the pressure is lower than necessary, the well depth can be decreased or its diameter increased, or both.

65 The pressure can also be reduced by placing in the well a small charge (such as one grain by weight) of a coarse powder, such as a nitro-cellulose-nitro-glycerin powder in the form of perforated cylinders of .035 inch diameter, .053 70 inch length and .007 inch perforation.

If it has been found necessary to change the dimensions of the base well any considerable amount, it may be necessary to revise the quantity of powder to give the required velocity, but with 75 a few experimental alterations in the amount of

powder and the depth and diameter of the base well, it is a very simple matter to secure the desired relations of velocity to pressure.

Ordinarily, the primer is not varied, either as to the charge or the size of the flash hole. 5 However, for varying primer charges and varying sizes of flash hole in the primer the procedure is to increase the depth and to decrease the diameter of the well as the primer charge increases or the flash hole decreases, and vice versa 10 for decreasing primer charge and increasing diameter of flash hole, until the relation of velocity and pressure is as required. If necessary, the main powder charge can be increased or decreased slightly to control the velocity by the 15 quantity of the powder, while the pressure is adjusted by the dimensions of the well.

In order to show graphically the effect of dimensioning the well with reference to the characteristic of the propellant employed and the 20 effect of grain size in the well, actual results will be given, together with the shell dimensions and granulations of the propellant.

In this test the shells were dimensioned (in inches) as follows:

| Shell  | Well diameter | Well depth | Flare diameters | Depth of steps |           |
|--------|---------------|------------|-----------------|----------------|-----------|
| Fig. 1 | .392          | .196       | .543—           | .675           | .196-.125 |
| Fig. 2 | .250          | .125       | .3—.4—.5—.565   | .075 Each      |           |
| Fig. 3 | .250          | .250       | .3—.4—.5—.565   | .075 Each      |           |
| Fig. 4 | .200          | .250       | .3—.4—.5—.565   | .075 Each      |           |

In this test the powder was a commercial fast burning shot gun powder (Hercules No. 2)—a nitro-cellulose-nitro-glycerin powder in the form of round flat discs of .055 inch diameter and .005 inch thickness and containing 30% of nitro-glycerin. In test No. 5 the well contained a coarse uncoated nitro-cellulose-nitro-glycerin powder 40 in the form of perforated cylinders of .035 inch diameter, .053 inch length and .007 inch perforation. The wadding was composed of felt wadding supplemented by hard wads.

Following are the results of the test for velocity and pressure:

| No.    | Shell  | Powder charge | No. of shots | Av. vel. | Av. max. pressure |    |
|--------|--------|---------------|--------------|----------|-------------------|----|
| Grains |        |               |              |          |                   |    |
| 1      | Fig. 1 | 28            | 100          | 867      | 10,470            | 50 |
| 2      | Fig. 2 | 28            | 100          | 888      | 9,529             |    |
| 3      | Fig. 3 | 32            | 100          | 933      | 9,420             |    |
| 4      | Fig. 4 | 34            | 100          | 947      | 8,780             |    |
| 5      | Fig. 4 | 37            | 30           | 970      | 7,600             | 55 |

An examination of the results will show that the velocity increases with the powder charge; in fact, the energy imparted to the shot charge by the propellant varies as the square of the velocity. Accordingly, as the powder charge is increased, the velocity square also increases. Now, ordinarily an increase in powder charge is accompanied by increase in maximum pressure. If, therefore, we should increase the powder charge in Figure 1 shell from 26 to 28 grains, while we can expect an increase in velocity, we can also expect an increase in the maximum pressure. An examination of the above results, however, shows that where the well has been 60 suitably dimensioned with reference to the characteristics of the propellant, then an increase in the powder charge, while accompanied by an increase in velocity, is actually accompanied by a decrease in maximum pressure. Thus, in the 70 75

shell, Figure 1, 26 grains of propellant, produce a velocity of 867 feet per second, at a pressure of 10,470 pounds per square inch. Where, however, the well has been reduced in diameter, as in Figure 2, then 28 grains of propellant, produce a velocity of 888 feet per second, at a pressure of 9,520 pounds per square inch. Moreover, when the well has been increased in depth, as between Figures 2 and 3, then 32 grains of propellant, 10 produce a velocity of 933 feet per second, at a pressure of only 9,420 pounds per square inch. Again, we find that reducing the diameter still further, as between Figures 3 and 4, an increased charge of 34 grains produces an increased velocity of 947 feet per second, but accompanied by a pressure of only 8,780 pounds per square inch. Test No. 5 shows the effect of employing a coarser grain propellant in the well. In this case 20 grains, including one grain (by weight) of coarse propellant, produced a velocity of 970 feet per second at a pressure of 7,600 pounds per square inch.

A comparison of the results is, indeed, striking. Thus, comparing shells, Figures 1 and 4, an increase of velocity of over 9% is actually accompanied by a decrease in the pressure of over 16%. As between tests 1 and 5, an increase in velocity of nearly 12% has been accompanied by an actual decrease in the maximum pressure of over 30 27%. This is extremely important in shot shells, in which, as previously stated, the powder charge is necessarily limited by the limiting breech pressure. The foregoing table shows that the powder charge can be actually increased from 30 to 42%, with resulting increases in velocities of from 9 to 12%, but with actual decreases in maximum pressures of from 16 to 27%.

The following are the results of tests obtained with a multiple piston gun, the readings being 40 taken at distances along the gun barrel, noted in inches. The shells and their powder charges are as in the preceding table. The number of shots fired was in each case ten, except for No. 5, in which there were only five shots fired.

| No. | Shell  | Average pressure at |       |      |      |      |      |      |      |      |      |
|-----|--------|---------------------|-------|------|------|------|------|------|------|------|------|
|     |        | 1"                  | 2"    | 3"   | 4"   | 5"   | 6"   | 7"   | 8"   | 9"   | 10"  |
| 50  | 1..... | 10860               | 9310  | 7970 | 6810 | 5045 | 4590 | 4390 | 4050 | 3800 | 3650 |
|     | 2..... | 10150               | 9590  | 8310 | 6340 | 5565 | 4865 | 4680 | 4390 | 4050 | 3800 |
|     | 3..... | 9930                | 10150 | 8925 | 7100 | 6270 | 5565 | 5135 | 4775 | 4495 | 4280 |
|     | 4..... | 9780                | 9820  | 9205 | 7520 | 6665 | 5810 | 5395 | 4955 | 4680 | 4390 |
|     | 5..... | 9310                | 9530  | 9640 | 8200 | 7160 | 6340 | 5730 | 5305 | 4865 | 4680 |

55 In Figure 5 the results have been plotted in the form of curves. These results illustrate the progressive burning action of the powder charge and the retardation of the initial combustion so that the maximum pressure is developed an extended distance along the gun barrel. The inertia of the shot charge is, therefore, overcome in such a manner that the shot charge is gradually moved out of the shell and along the barrel, but the pressure is sustained an extended distance along the gun barrel. While the differences may not at first sight be striking, it must be remembered that an increase of pressure of 740 pounds per square inch as between Nos. 1 and 4, and 1030 as between Nos. 1 and 5, ten inches along the gun barrel, has an important effect upon the velocity, especially when we keep in mind that the maximum pressure is not increased but, in fact, materially decreased. The work done is represented by the area of the diagrams below the curves, and it will be readily seen that these

areas are considerably greater in shells loaded in accordance with this invention than where the shell base is not provided with a well dimensioned to secure control of the pressure and ballistic properties.

From a consideration of Figure 5, it will be seen that curve No. 1, corresponding to shell, Figure 1, has a sharp peak while the pressure drops rapidly, thereby showing that the initial combustion is not retarded substantially. The pressure attending 10 the employment of 26 grains of powder in shell No. 1 also indicates that the charge is about the desired maximum charge of the particular fast burning nitro-cellulose-nitro-glycerin powder employed. As, however, the well diameter is decreased or/and the depth increased from 1 through 2, 3 and 4, it will be seen that the curve rapidly changes its configuration and flattens out, not only at the peak but also along the gun barrel. This would seem to indicate that for a given 20 propellant there is a rather definite zone or field of dimensions, where a decrease in the diameter or an increase in the depth of the well becomes effective to retard the initial combustion substantially and to reduce the maximum pressure sub- 25 stantially. The dimensioning of the well is, of course, with reference to the particular propellant employed; but, as pointed out above, the proper proportions can be readily arrived at by first determining the charge required to produce 30 the desired velocity and by then varying the well diameter or/and depth until the pressure developed is within the desired limits.

From the data given in the specification it will be seen that a shot shell having a base wad 35 provided with a powder receiving well will attain the objects of this invention if it has the following characteristics: if the well diameter is not less than 0.10 inch in order to receive powder grains of practical dimensions; if this well diameter is not greater than 0.30 inch and preferably between 0.20 and 0.25 inch; if the minimum depth of the well is 0.05 inch plus 0.66 times its diameter and is preferably between 0.20 and 0.25 inch; the maximum depth of the well is, of course, determined by the depth of the base wad which is limited in all shot shells by the length of the shell and is generally fixed by the shot charge, the wadding and the required powder charge. It will, of course, be understood that the 50 term "shot shell" is a term well understood by those skilled in the art as meaning a shell having a primer, a powder charge, a shot charge and, of course, wadding between the powder and shot charges.

55 It will, therefore, be seen that this invention accomplishes its objects. A shot shell is produced having improved characteristics as distinguished from those of the prior art, and this result is secured in a simple and effective manner. While the invention is particularly applicable to the general type of cartridge as shown and described, it will be understood that this invention is applicable in many cases to other forms and types of cartridges. It will, furthermore, be understood that, while certain theories have been advanced, this has only been done to facilitate the explanation; for this invention is not limited to any particular theory. It will, furthermore, be understood that certain features, operations 65 and sub-combinations are of utility and may be employed without reference to other features, operations and sub-combinations. That is contemplated by and is within the scope of the appended claims. It is, furthermore, obvious that 75

various changes may be made in details and operations, within the scope of the appended claims, without departing from the spirit of this invention. It is, therefore, to be understood that this 5 invention is not to be limited to the specific details and operations shown and/or described.

Having thus described the invention, what is claimed is:

1. A loaded shot shell having a primer and a 10 propellant charge, the base of the shell having a well containing coarser grained propellant than the remainder of the charge.

2. A loaded shot shell having a primer and a propellant charge, the base of the shell having 15 a well containing coarser grained propellant than the remainder of the charge and the well being dimensioned to control the ballistics of the shell.

3. A shot shell having a base wad provided with a powder-receiving well whose diameter is 20 not less than 0.10 inch and not greater than 0.3 inch and whose minimum depth is 0.05 inch plus 0.66 times its diameter.

4. A shot shell having a base wad provided with a powder-receiving well whose diameter is be-

tween 0.2 and 0.3 inch and whose minimum depth is 0.05 inch plus 0.66 times its diameter.

5. A shot shell having a base wad provided with a powder-receiving well whose diameter is between 0.20 and 0.25 inch and whose minimum 5 depth is 0.05 inch plus 0.66 times its diameter.

6. A shot shell having a base wad provided with a powder-receiving well whose depth is about .25 inch and whose diameter is .20 to .25 inch.

7. A loaded shot shell having a base wad, a 10 primer therein, a well in front of said primer, the diameter of said well being not less than 0.10 inch and not greater than 0.3 inch and the minimum depth of said well being 0.05 inch plus 0.66 times its diameter, and a powder charge in said 15 shell and in said well.

8. A loaded shot shell having a base wad, a primer therein, a well in front of said primer, the diameter of said well being not less than 0.10 inch and not greater than 0.3 inch and the minimum depth of said well being 0.05 inch plus 0.66 times its diameter, and a charge of fast burning 20 powder in said shell and in said well.

WILLIAM E. WAGNER.